

Sept. 5, 1944.

A. S. MOORE

2,357,420

APPARATUS FOR GALVANIZING RODS

Filed Dec. 2, 1942

2 Sheets-Sheet 1

Fig. 1.



Sept. 5, 1944.

A. S. MOORE

2,357,420

APPARATUS FOR GALVANIZING RODS

Filed Dec. 2, 1942

2 Sheets-Sheet 2



## UNITED STATES PATENT OFFICE

2,357,420

## APPARATUS FOR GALVANIZING RODS

Allen S. Moore, Lebanon, Pa., assignor to Bethlehem Steel Company, a corporation of Pennsylvania

Application December 2, 1942, Serial No. 467,618

10 Claims. (Cl. 91—59.4)

My invention relates to an apparatus for coating uniformly rod-like or tubular objects, and more particularly it relates to an apparatus for the uniform and economical galvanizing of metallic sucker rods.

Oil well sucker rods of the double pin and coupling type are straight steel rods, usually 25 or 30 feet long, having upset and externally threaded ends or pins to which the couplings are attached to form a part of a pumping string. In some wells the presence of corrosive fluids has heretofore made it necessary to use high-grade steels employing rather costly alloying elements, such as molybdenum, chromium, manganese and nickel, which are now under war priorities and practically unobtainable. For very deep or highly corrosive wells, there is at present no satisfactory substitute for the high strength and corrosion resistance of these alloy steels, but galvanized rods of ordinary carbon steel may serve quite successfully under less extreme conditions, provided only that the protective zinc coating is as strongly adherent and ductile and as uniform in thickness as possible.

There are two methods of galvanizing in common use, viz., the electrogalvanizing process and the hot-dip process. The cold coating applied by an electrolytic process is generally uniform, when well applied, and the thickness is easily regulated by varying either the current density or the time of deposit, but the reduction in output compelled by the time factor, and the requirements of expensive electrical equipment and current, make this process uneconomical commercially.

Zinc coatings applied by the hot-dip process, on the other hand, are relatively free of the type of porosity caused by the tiny pores or pinholes which are often found in electrolytic coatings, and are cheap and quick and easy to apply. But as the threaded rods emerge from the galvanizing pan, some of the zinc they carry remains in the molten state for a brief period, and, unless prevented from doing so, tends to flow downward on the surface of the rod, making the coating rough and uneven and filling the roots of the threads with spelter. Such a coating represents an actual waste of zinc, for the durability of an unevenly applied coating is determined by the thinnest part of the coating and not by the thickest part.

Any defect or deficiency in the zinc coating will permit quick rusting, even before use, and very badly rusted threads can obviously destroy all the usefulness of the rod, for the making up

of rusted threads may result in thread galling and imperfect shouldering of the joint. Surplus zinc in the threads will interfere with attaching couplings, so that when the threads are clogged with zinc the only way to obtain usable threads is to "bump" them, i. e., to rap or knock them against a hard surface to remove the excess spelter. This additional step means extra expense and labor and may even shorten the life of the rod, for undue hammering may deform the thread or cause cracks that radiate out from the point of the blow and extend for considerable depths below the surface. A smooth, uniform coating over the threads and body of the rod is thus about the best obtainable insurance against early operating failure of a string of galvanized sucker rods.

With perhaps less direct force, similar considerations apply to galvanized coatings on other rod-like or tubular objects, such as pipes and the like.

One object of this invention, therefore, is an apparatus for producing a hot-dip galvanized coating which will be smoothly and uniformly distributed over the galvanized article.

Another object is an apparatus for procuring more evenly and completely coated threads.

Still another object is an apparatus adapted for covering rod-like or tubular articles of metal with a tighter and more ductile zinc coating which will not flake or crack off under stress.

Other and further objects will appear hereinafter in the specification and appended claims.

Having thus given a general description of the advantages and objects of my invention, I shall now in order to make the same more clear, refer to the annexed two sheets of drawings forming a part of this specification, and in which like characters of reference indicate like parts.

Figure 1 is a side elevation of the apparatus of my invention, and showing its relation to the galvanizing and quenching tank;

Fig. 2 is a top plan view thereof;

Fig. 3 is a front elevation showing in detail the self-adjusting guide roller device which permits the passage of the enlarged portions of the sucker rods;

Fig. 4 is a side elevation of the guide roller device shown in Fig. 3; and

Fig. 5 is a horizontal section of a portion of the mounting of the guide roller device taken on the lines 5—5 of Figure 4.

Referring now to the various characters of reference on the drawings, the numeral 1 indicates a sucker rod, 2 one end of a conventional

galvanizing tank, which is a long shallow pan filled with molten zinc or spelter, 3 a base mounted in skewed relation at the exit end of said tank, 4 an electric motor fastened to the base, 5 the drive shaft of the motor, 6 a pinion on shaft 5, and 7 an engaging gear mounted on and driving a shaft 8. Said shaft 8 drives through gears 9, 10 and 11 the magnetic rolls 12 and 13 journaled in bearings 14, 15, 16 and 17 in end mountings 18 and 19. The magnetic flux which magnetizes said rolls emanates from the magnetic coils 20 and 21, activated by any suitable source of direct current electricity, and enclosing the steel core 22.

In alignment with the galvanizing tank 2 and near the diagonal ends of the skewed magnetic rolls 12 and 13 are located the hollow air rings 23 and 24, drilled with a plurality of evenly spaced holes on their inner peripheries directed at an angle of about 45° toward the advancing sucker rod 1, and mounted on fittings 25 which are preferably of brass or copper or the like to insulate from stray magnetic flux. Said fittings 25 and 26 connect through pipe 27 equipped with valve 28 to any suitable source of heated and compressed air (not shown). As the galvanizing tank 2 will be kept heated in the usual practice by a series of gas flames (not shown) within side burner compartment 29, the air under pressure may be heated conveniently, for example, by running the connecting pipe 27 from the compressor or other source through said gas flames, or if desired, through the molten spelter itself.

To insure the proper direction and contact of the rod 1 as it rotates and moves forward over the rolls 12 and 13, a guide device is provided which comprises a pair of mountings 30 of brass or other non-magnetic metal secured by bolts 31 to the base 3, between said rolls 12 and 13, and having grooved slideways 32 to permit a limited amount of vertical movement to perforated blocks 33 keyed thereto and normally held in place by vertical threaded rods 34, springs 35, and adjusting nuts 36. Said blocks 33 are connected by a transverse shaft 37, held in place by cotterpins 38 and having mounted thereon a grooved idle roller 39.

Adjacent thereto is the conventional elongated quenching tank 40, on which is mounted the incline 41 and pivoted conveyor trough 42, the latter being provided with a plurality of aligned idle rollers 43 like the one shown and an end stop (not shown) which may actuate an automatic kicker (also not shown) to dump the galvanized rod 1 into the quenching tank 40.

In the operation of my invention, any traces of rust and mill scale which may be present on the rods 1 are removed by pickling in a hot dilute acid solution, and washing with clean water. Then the rods 1 are fluxed in a hot solution of zinc ammonium chloride, and dipped into the molten spelter in the galvanizing tank 2. The spelter is kept at a temperature between 790° F. and 870° F., the period of immersion therein being determined by the size of the rods and the weight of zinc coating desired, and the rods are kept from contact with the pasty zinc iron dross which collects upon the bottom of the galvanizing tank 2 by resting in a suspended cradle (not shown).

With tongs or a forked lever arrangement (not shown) the rods 1 are started one at a time by hand through the first air ring 23 until the rod 1 makes contact with the magnetic driven rolls 12 and 13. The self-adjusting guide roller

39 midway between the two magnetic rolls 12 and 13 insures the proper direction and contact of the rod as it rotates and moves forward over said rolls 12 and 13.

5 The rotation of the rolls 12 and 13 then carries the rod 1 forward through the second air ring 24 up the incline 41 over the rollers 43 onto conveyor trough 42. Air is blown from the air rings 23 and 24 at a pressure of 25 to 80 pounds per square inch, and is preheated to a temperature high enough to prevent too rapid cooling of the zinc. The variation of air pressure and temperature controls the thickness of the zinc coating on the rod and can be regulated to suit the number of Preece dips required.

10 The speed of the rod carries it against a stop at the end of the conveyor trough 42, where a kicker arrangement (not shown) operated automatically or by hand discharges the rod into 20 the water quenching tank 40. The coating is hardened and brightened by this quenching operation. The galvanized rods are then lifted by hand from the quenching tank 40 and further processed for shipment.

15 The spinning of the galvanized rods in this manner results in a very uniform coating. Rods which have not been spun show coatings of excessive thickness on their lower surfaces, due to gravity, and thin and inadequate coatings on 25 their upper portions. The combination of the air rings with the spinning action of the skewed rolls automatically and quickly removes excess spelter from the threaded ends, and eliminates the extra step and added labor of cleaning the 30 threads by bumping.

35 An even more important advantage is that the coating produced is a great deal more adherent and ductile than any hot-dip coating for sucker rods heretofore known. Rods galvanized according to my invention have been subjected to repeated and severe tensile tests without the coating flaking or cracking off, and even a 180° bend test gave only minor cracks in the coating which were not especially detrimental 40 because of the nature of the protection afforded by the electropositive zinc coating.

45 Although I have thus shown and described my invention in considerable detail, I do not wish to be limited strictly to the exact and specific details shown and described, but I may also use such substitutions, modifications, or equivalents thereof as are embraced within the scope of the invention or as are pointed out in the appended claims.

50 Having thus described my invention, what I claim as new and useful and desire to protect by Letters Patent is:

55 1. An apparatus for producing uniform ductile coatings on rods and the like coated with molten metal, comprising a plurality of aligned air rings for smoothing the coating and making uniform the coating thickness, and means for rapidly advancing and spinning the rod through the air rings.

60 2. An apparatus for producing uniform ductile coatings on rods and the like coated with molten metal, comprising a plurality of aligned air rings for uniformly removing excess metal and rendering the remainder smooth and even, and conveying mechanism adapted to spin the rod in the course of travel in a line substantially coinciding with the center of the air rings.

65 3. An apparatus for producing uniform ductile coatings on rods and the like coated with molten metal, comprising a plurality of driven rolls hav-

ing their axes inclined to the line of travel of the coated rod, and aligned hollow rings on said line of travel for delivering air streams upon said coated rod to wipe excess coating metal therefrom.

4. An apparatus for producing uniform ductile coatings on rods and the like coated with molten metal, comprising a plurality of magnetic rolls having their axes skewed in relation to the direction of travel of the coated rod, means for rotating said rolls, means for supplying a heated fluid under pressure, and means for directing said fluid under pressure against and around the periphery of the coated rod.

5. An apparatus for producing uniform ductile coatings on rods and the like coated with molten metal, comprising a plurality of hollow rings perforated and adapted for directing jets of fluid with substantial uniformity about the circumference of the rod, and spinning and conveying means comprising a series of skewed driven rolls one or more of which are magnetized.

6. An apparatus for producing uniform coatings on threaded rods and the like coated with molten metal, comprising a pair of spaced air rings suitably perforated for delivering a stream of air onto the coated surface at an angle of approximately 45° to the plane of said surface to wipe excess coating metal therefrom, a pair of skewed driven rolls therebetween each having a magnetizable periphery, coil windings in alignment with said rolls, a magnetic circuit energized by said coil windings and including said rolls, and guide means for insuring the proper contact and direction of the coated rod as it is rotated and advanced by the rolls.

7. An apparatus for producing uniform coatings on hot-metal coated sucker rods or the like, comprising a pair of skewed magnetic rolls for advancing and spinning the coated sucker rods, a pair of adjacent air rings for smoothing and evening the coating on the sucker rods, an idle roller for directing the sucker rods through the air rings, and means for manually adjusting the idle roller to accommodate different sizes of sucker rods.
8. An apparatus for producing uniform ductile coatings on rod-like metal articles comprising a pair of aligned air rings, and a pair of skewed driven magnetic rolls situated therebetween.
15. An apparatus for producing uniform ductile coatings on rod-like metal articles comprising a pair of aligned hollow rings adapted for the passage therethrough of the coated article, each of said rings having a circular series of openings 20 directed toward the article, means for supplying a heated fluid air to the pair of hollow rings, and a pair of driven magnetic rolls situated between the aligned hollow rings in skewed relation thereto for simultaneously rotating and conveying the rod-like article through the rings.
10. An apparatus for producing uniform ductile coatings on hot-dip galvanized sucker rods comprising a pair of aligned air rings, a pair of motor driven magnetized rolls skewed with respect to the common center line of the air rings 30 and placed between said air rings for spinning the rods while advancing said rods therethrough, and an idle guide roll placed between and above the magnetized skew rolls to assist in aligning the rods passed through the apparatus.

ALLEN S. MOORE.